

**3,795,519**  
**PHOTOGRAPHIC MATERIALS CONTAINING**  
**MORDANTS**

MORDANT'S

Takushi Miyazako, Tatsuya Tajima, Hirotetsu Kato,  
Tadayoshi Kokubu, Tsutomu Nishina, and Nobuo  
Tsuij, Minami-ashigara, Japan, assignors to Fuji Photo  
Film Co., Ltd., Kanagawa, Japan  
No Drawing. Filed July 24, 1972, Ser. No. 274,373  
Claims priority, application Japan, July 30, 1971,

46/57,276  
Int. Cl. G03e 1/84

**U.S. Cl. 96—84 A**

## 12 Claims

## ABSTRACT OF THE DISCLOSURE

A photographic material comprising a support having thereon a hydrophilic colloid layer containing a polymer of an addition product of bisacrylamide and a secondary diamine or the quaternary salt thereof, and a water-soluble acidic dye is disclosed.

## BACKGROUND OF THE INVENTION

(1) Field of the invention

This invention relates to mordants for use in colored layers in photographic materials.

## (2) Description of the prior art

It is well known to provide colored layers for the purpose of light filtering or light absorbing. The position of the colored layer in the photographic material depends upon its purpose. The colored layer may be coated as the outermost layer when overall filtering is required, between layers when selective filtering is required or next to the support for antihalation purposes.

These layers often contain organic dyes, but these dyes often exert a deleterious effect on the light-sensitive layers used in the photographic material. Therefore, it is important to prevent these dyes from diffusing into adjacent layers.

As a means to prevent this diffusion, a method of converting a fairly soluble dye into an insoluble complex using a mordant is well known. For example, an acid dye can be mordanted with a high molecular weight compound having a basic group. By the way, where light filtering or light absorbing layers are used in photographic materials, it is necessary that these layers be bleached during the photographic processing. For example, the dye must be released from the mordant and discharged from the layer by immersing the photographic material in an alkaline solution, such as a photographic developer solution.

Processes utilizing mordants, such as are described above, are disclosed in a great number of patents, e.g., British Pats. Nos. 786,592, 906,083 and 1,162,214; U.S. Pat. No. 3,445,231; German Pats. OLS 1,914,361 and 1,914,362, etc.

However, in the processes which have been proposed so far, the dye is not sufficiently discharged in many cases which results in the color remaining. In addition, a considerable amount of thiosulfate ions are absorbed from an acidic fixing solution due to the mordanting action of the mordant to acidic compounds, the mordant remaining in the layer, and this results in reducing the stability of the image formed on the material.

An object of the present invention is to provide compounds which can be used as mordants for acidic dyes whose mordanting action is markedly reduced due to the action of alkaline solutions.

## SUMMARY OF THE INVENTION

The present invention provides photographic materials comprising a support having thereon a hydrophilic colloid layer containing an addition polymer of bisacrylamide and a secondary diamine, or the quaternary salt thereof, and a water-soluble acidic dye.

## DETAILED DESCRIPTION OF THE INVENTION

10 The addition polymer of bisacrylamide and a secondary diamine used as the mordant in the invention is a polymer, of repeating units, in which an amino group of the secondary diamine is added to the terminal unsaturated double bond of the bisacrylamide. The nitrogen atom of this amino group of the secondary diamine exists as a tertiary amine in the polymer, and the term 15 "quaternary salt thereof" as used herein means the conversion of such a tertiary amine to the quaternary salt.

The term bisacrylamide, which is used as the starting material for the mordants in accordance with the present invention, includes compounds represented by the following General Formula I:



wherein  $R_1$  and  $R_2$ , which may be the same or different, each represents a hydrogen atom, a methyl, an ethyl or a propyl group, and  $A$  represents an alkylene group having from 1 to 6 carbon atoms, which may be substituted with a methyl or an ethyl group.

Specific examples of the compounds represented by the General Formula I are illustrated hereinafter.



The other starting material, the secondary diamine, includes piperazine, ( $C_1$  to  $C_4$ ) alkyl-substituted piperazine and  $N,N'$ -di-( $C_1$  to  $C_4$ )alkylethylenediamine. As specific compounds, there are illustrated piperazine, 2,5-dimethyl-piperazine,  $N,N'$ -dimethylethylenediamine,  $N,N'$ -diethyl-ethylenediamine and the like.

The polymer can readily be synthesized by heating the bis-acrylamide and the secondary diamine in water. The quaternary salt thereof also can be synthesized readily

in any conventional manner, i.e., by the reaction of an alkyl halide (e.g., ethyl bromide, butyl bromide, etc.) or an alkylsulfate (e.g., diethyl sulfate, etc.) with the tertiary amine group of the polymer.

Specific processes for synthesizing these polymers are illustrated hereinafter. The intrinsic viscosity of the resulting polymer is that measured in a 1% sodium chloride aqueous solution at a temperature of 30° C.

#### SYNTHESIS EXAMPLE 1

25.5 grams (0.165 mol) of methylenebisacrylamide and 32.0 g. (0.165 mol) of piperazine (6 hydrate) were dissolved in 10 ml. of water and stirred for 5 hours maintaining the temperature at 40–50° C. After leaving the reaction mixture overnight at room temperature, acetone was added to precipitate the polymer formed. The polymer was then collected and dried. Thus, 35 g. (88% yield) of a polymer having an intrinsic viscosity of 0.608 were obtained. The resulting polymer is considered to contain repeating units of the following formula.



#### SYNTHESIS EXAMPLE 2

In the same manner as described in Synthesis Example 1, there was obtained 20 g. (91% yield) of a polymer using 15.4 g. (0.1 mol) of methylenebisacrylamide and 17.5 g. (0.09 mol) of piperazine 6H<sub>2</sub>O. The resulting polymer had an intrinsic viscosity of 0.15.

#### SYNTHESIS EXAMPLE 3

In the same manner as described in Synthesis Example 1, there was obtained 22 g. (86% yield) of a polymer using 18.2 g. (0.1 mol) of methylenebisacrylamide and 19.4 g. (0.1 mol) of piperazine 6H<sub>2</sub>O. The resulting polymer had an intrinsic viscosity of 0.52.

#### SYNTHESIS EXAMPLE 4

In the same manner as described in Synthesis Example 1, there was obtained 21 g. (82% yield) of a polymer using 18.2 g. (0.1 mol) of methylenebisacrylamide and 17.5 g. (0.09 mol) of piperazine 6H<sub>2</sub>O. The resulting polymer had an intrinsic viscosity of 0.124.

#### SYNTHESIS EXAMPLE 5

In the same manner as described in Synthesis Example 1, there was obtained 23 g. (85% yield) of a polymer using 15.4 g. (0.1 mol) of methylenebisacrylamide and 11.6 g. (0.1 mol) of N,N'-diethylethylenediamine. The resulting polymer had an intrinsic viscosity of 0.63.

#### SYNTHESIS EXAMPLE 6

In the same manner as described in Synthesis Example 1 there was obtained 23 g. (86% yield) of a polymer using 15.4 g. (0.1 mol) of methylenebisacrylamide and 11.4 g. (0.1 mol) of 2,5-dimethylpiperazine. The resulting polymer had an intrinsic viscosity of 0.48.

#### SYNTHESIS EXAMPLE 7

10 grams of the polymer obtained in Synthesis Example 1 and 6.4 g. of diethyl sulfate were stirred together with 100 ml. of dimethylformamide for 12 hours. Thereafter, the dimethylformamide was removed under reduced pressure, and the residue was placed in a cellulose tube to conduct dialysis overnight, then was lyophilized. Thus, there was obtained 12 g. of a polymer having an intrinsic viscosity of 0.75. The resulting poly-

mer is considered to contain the following repeating units.



The mordants in accordance with the present invention have the property that they very rapidly lose their mordanting ability to acidic dyes due to the action of an alkaline solution. Accordingly, they have an important characteristic that, when incorporated in a filter layer or an antihalation layer of a photographic light-sensitive material, the dye mordanted by them can be released easily due to the action of an alkaline photographic processing solution and thus no color remains in the layer.

When the molecular weight of the polymer of the invention is too low, the polymer itself tends to diffuse into the material, whereas, when the molecular weight is too high, compatibility with hydrophilic colloids becomes poor. Therefore, polymers having an intrinsic viscosity of from about 0.01 to 3.0, preferably, about 0.1 to 1.5 is suitable, this intrinsic viscosity being measured at 30° C. using a 1% sodium chloride aqueous solution.

The photographic material of the present invention comprises a support material having thereon at least one hydrophilic colloid layer containing a mordant of the invention, which layer may also contain a light-sensitive silver halide, or, the light-sensitive photographic material may comprise a support having thereon at least one hydrophilic colloid layer containing a mordant of the invention and at least one light-sensitive silver halide emulsion layer. The light-screening or antihalation layers containing the mordant can be prepared by coating an aqueous solution comprising a mordant of the invention, an acidic dye, a hydrophilic colloid binder and a coating aid such as saponin, sodium alkyl benzenesulfonate, polyoxyethylene alkylphenyl ether, etc. on the support or on a photographic layer. In order to improve the strength of the light-screening or antihalation layer, compounds such as formaldehyde, mucochloric acid, chlorotriazine derivatives, etc. can also be added as a hardening agent for the colloidal binder. The proportions of mordant, dye, colloidal binder, hardener and coating aid can be varied over a wide range and will depend upon the specific requirements of the photographic material to be produced. The methods used to determine the optimum compositions are well known to those skilled in the art and require no further detailed explanation here.

The support materials include any of those usually used in the field of photography, such as cellulose acetate, cellulose propionate, polyesters, polystyrene, polypropylene, paper or polyethylene-coated paper.

Suitable hydrophilic colloid materials which can be used include gelatin, albumin, collodion, gum arabic, agar-agar, cellulose derivatives (e.g., the alkyl esters of carboxylated cellulose, hydroxyethyl cellulose, carboxymethyl hydroxyethyl cellulose, etc.), synthetic resins (e.g., polyvinyl alcohol, polyvinyl pyrrolidone, etc.) and others well known in the art.

The dyes that can be effectively mordanted in accordance with the invention are those having at least one acidic group such as a sulfo group or a carboxy group, including for example, the oxonol dyes, the styryl dyes, the azo dyes, the triphenylmethane dyes, the cyanine dyes, or the merocyanine dyes. Specific examples of such dyes are described in U.S. Pats. Nos. 3,316,091, 3,423,207, 3,445,231; British Pats. Nos. 506,385, 906,083, 993,466, 1,034,044, 1,142,697, 1,162,214; French Pat. No. 1,421,679; German Offenlegungsschrift Nos. 1,472,789, 1,547,999; Belgian Pats. Nos. 689,044 and 697,267. However, the invention is not limited to just those dyes described above and any dye containing one or more sulfo

or carboxyl groups can be employed, for example, 2,5-bis(sulfophenyl)thiazolo[5,4-d]thiazole, 3-phenyl-2-phenylimino-5-(2-sulfobenzol)-4-thiazolidone and uranine.

Typical examples of suitable dyes are illustrated below.

Dye 1



Dye 2



Dye 3



Dye 4



Dye 5



Dye 6



Dye 7



Dye 8



or

Dye 9



The silver halide light-sensitive emulsion layers can contain silver halides such as silver chloride, silver bromide, silver iodide, silver chlorobromide, silver bromoiodide, silver chlorobromoiodide, etc. as the light sensitive material. The silver halide emulsion may be sensitized using any of the sensitizers conventionally used.

The filter layer or antihalation layer containing a mordant of the invention provides an excellent photographic material as will be illustrated in the following examples. The mordant of the invention can also be used for preparing excellent image-receiving layers for use in the dye-transfer process.

The present invention will be illustrated in greater detail by reference to the following examples.

#### EXAMPLE 1

8 ml. of a 5% aqueous solution of the polymer obtained in Synthesis Example 1 was added to an aqueous solution comprising 50 ml. of water, 5 g. of gelatin, 0.1 g. of saponin and 0.1 g. of mucochloric acid, then 10 ml. of a 2% aqueous solution of each of Dyes 1, 4 and 6 was added thereto. Thereafter, the pH of the solution was adjusted to 6.5 with a 1 N sodium carbonate aqueous solution, and water was added to adjust the total volume to 100 ml.

For comparison, a solution not containing the polymer was prepared in exactly the same manner as described above. Samples were prepared by applying each of these dye containing solutions so obtained to a clear under-coated film base of cellulose triacetate in a dry thickness of 2 microns, then coating thereon a fine-grained silver chlorobromide emulsion containing 40 mol percent of panchromatically and spectrally sensitized silver chloride and 120 g. of gelatin per 1 mol of silver halide in a dry thickness of 2 microns, and further coating thereon a protective layer of gelatin in a dry thickness of 1 micron.

Furthermore, a sample comprising only the emulsion layer and the protective layer was prepared for comparison.

These samples thus prepared were wedge-exposed and were developed and fixed in a conventional manner. Samples containing the dyes were completely bleached.

Comparing the photographic sensitivity of each sample with each other, the sensitivity of the samples containing



N,N'-dimethylethylenediamine or N,N' - diethylethylenediamine.

7. The photographic material as claimed in claim 2, wherein said bisacrylamide compound is methylenebisacrylamide and wherein said secondary diamine is piperazine.

8. The photographic material as claimed in claim 2, wherein said bisacrylamide compound is methylenebis-methylacrylamide and wherein said secondary diamine is piperazine.

9. The photographic material as claimed in claim 2, wherein said bisacrylamide compound is methylenebis-acrylamide and wherein said secondary diamine is N,N'-diethylethylenediamine.

10. The photographic material as claimed in claim 1, wherein said hydrophilic colloid is gelatin.

11. The photographic material as claimed in claim 1, wherein said water-soluble acidic dye is

Dye 1



Dye 2



Dye 3



Dye 4



Dye 5



5

10

Dye 6



15

Dye 7



20

Dye 8



35

Dye 9



40

or Dye 9



45

12. The light-sensitive photographic material as claimed in claim 1, wherein said support has thereon at least one light-sensitive silver halide emulsion layer.

50

55

## References Cited

## UNITED STATES PATENTS

- |    |           |        |                            |         |
|----|-----------|--------|----------------------------|---------|
| 60 | 2,675,316 | 4/1954 | Carroll et al. -----       | 96-84 A |
|    | 3,184,309 | 5/1965 | Minsk et al. -----         | 96-84 A |
|    | 3,234,025 | 2/1966 | Van Hoof et al. -----      | 96-84 A |
|    | 3,741,768 | 6/1973 | Van Paesschen et al. ----- | 96-84 A |

RONALD H. SMITH, Primary Examiner

65

U.S. Cl. X.R.

96-84 R, 114